

## UNITED STATES PATENT OFFICE

1,990,650

## HEAT RESISTANT ALLOY

Hans Jaeger, Milwaukee, Wis., assignor to A. O.  
Smith Corporation, Milwaukee, Wis., a corpora-  
tion of New York

No Drawing. Application June 25, 1932,  
Serial No. 619,358

## 14 Claims. (Cl. 75—1)

The invention relates to alloy steels which contain relatively large amounts of aluminum and it is among the objects of the invention to provide steels which have a high ohmic resistance and great resistance to deterioration or scaling especially at high temperatures, and to provide resistant steels of the kind so that they can be practicably worked or forged into shapes, sheets, wires or ribbons. Another object of the invention is to provide resistance elements composed of these alloys which are suitable and durable when they are used at moderately high temperatures.

In accordance with the invention, the alloys may be considered generally as high aluminum—low carbon—chromium steels which contain small amounts of other elements that give the steels properties suiting them for use as heating elements and for manufacturing purposes. The alloys contain small amounts of silicon, from about 5% to 10% chromium and about 16% to 20% aluminum. The alloys are heat resistant and are especially suitable for making electrical resistance elements when they contain suitable amounts of modifying elements because of their durability and high ohmic resistance.

It was found that steels of this aluminum content are not workable into the desired shapes for heating elements if they contain more than about 0.05% carbon and that more than this amount of carbon is prohibitive in manufacturing attenuated articles from the alloys which are to be used for heating elements. Although carbon is commonly present in the alloys, they may be free from carbon. For the best results, the carbon should be as low as possible and not over 0.05% carbon.

The alloys of iron, chromium and aluminum are not well adapted for fabricating attenuated articles unless they are modified by small additions of other elements which will be hereinafter described. Without additional or modifying elements, the forgeability of alloys which contain even less than 16% aluminum is not satisfactory for manufacturing purposes while those which contain more than 16% are practically unforgeable without the additions. With more than about 20% aluminum, the workability and resistance to oxidation at high temperatures are not good in that the alloys lack cohesion at the grain boundaries. About 5% to 10% chromium improves the workability of the alloys, but in those which contain more than about 8.5% chromium and 16% of aluminum, the chromium is not effective and larger amounts of chromium lower the ohmic resistance and the resistance to scaling.

The high aluminum alloys machine poorly if they contain more than about 8% chromium.

The best results are obtained when the alloy is carefully deoxidized. Silicon is commonly present either as an impurity in the materials used for making the alloys or as a residue of the deoxidizer. Fractional percentages of silicon are desirable in that they improve the resistance to scaling but not more than about 0.25% may be present. Larger amounts of silicon decrease the forgeability.

Even smaller amounts of silicon than 0.25% decrease the forgeability unless one or more effective grain refining elements are added. Titanium and molybdenum have been found to be effective grain refining elements. About 0.1% to 0.5% of the grain refiner is used. Molybdenum can be used for this purpose instead of titanium, but it may desirably be present in addition to titanium since it strengthens the grain refining action of titanium. Increased amounts of molybdenum up to about 1.5% are beneficial in that these amounts increase the ohmic resistance. The highest resistances can desirably be attained by additions of 1.0% to 1.5% molybdenum, but these alloys are suitable for use only at temperatures below about 1200° C. since loss of molybdenum is noticeable at higher temperatures, such as 1400° C. Molybdenum in amounts of 0.5% to 1.5% in conjunction with manganese in amounts of about 0.5% to 1.5% gives the alloys practically a zero temperature coefficient of resistance. From considerations of scaling, forgeability, ohmic resistance and temperature coefficient of resistance, the combination of about 0.5% to 1.0% manganese and 0.5% to 1.0% molybdenum with or without titanium may be mentioned as a desirable range.

I have found that alloy heating elements containing more than 16% to about 20% aluminum, about 5% to 8.5% chromium, about 0.1% to 0.5% titanium and about 0.1% to 1.0% molybdenum give excellent workability and resistance to scaling. In the alloys containing this aluminum content the titanium is essential for ready workability and the molybdenum adapts the alloys to practicable shop conditions. Materially more than 0.5% of titanium decreases the ohmic resistance, and more than 1.5% of molybdenum makes the alloys non-workable and non-machinable.

An addition of about 0.4% to 1.5% of manganese will give a practically zero temperature coefficient of resistance. Larger amounts of manganese lower the resistance to scaling. The best results are not obtained when the highest amounts

of both chromium and manganese are present. Therefore, smaller amounts of manganese may be used with the highest chromium contents and smaller amounts of chromium may be used when 5 higher contents of manganese are present.

A representative ingot containing 17.5% aluminum, 8.5% chromium, 0.44% manganese, 0.36% titanium, 0.02% carbon, 0.13% silicon and the remainder iron with small fractional amounts 10 of sulphur and phosphorus was found to have excellent forging properties when the casting was made in a mold, such as a sand mold, in which chilling was avoided. Ribbon was made from the ingot by hot forging and rolling. These ribbons 15 were used for heating elements by passing current therethrough. The alloy had practically a zero temperature coefficient of resistance. The resistance of the elements was about 220 microhms per cubic centimeter at 25° C. and they 20 showed excellent durability and freedom from scaling when they were heated to 1200° C. for long periods of time. Other alloys, which were similar except that in addition to titanium, they contained molybdenum from 0.5% to about 1.0%, 25 were easier to work when cast under the same conditions and they had excellent forging properties when some chilling was present in the mold. An increase of carbon to 0.25% or silicon to 0.5% made the alloys unforgeable. An increase of the 30 chromium to 9.5% made the alloy unforgeable or so difficult to forge that it was impracticable to apply it to the manufacture of attenuated heating elements.

High ohmic resistances are found in the alloys 35 containing more than 16% up to 18% aluminum, namely 200 to 240 microhms per centimeter cube. This resistance is about twice that of alloys containing approximately 80% nickel and 20% chromium. Comparative tests with the chromium-nickel heating elements showed that the 40 above described heating elements lost less than half as much by scaling when they were heated to temperatures of about 1400° C. in air. The chromium-nickel elements became pitted and 45 dull in appearance whereas the described elements remained smooth and retained a light gray color.

Although the limiting proportions of the various constituents are specifically recited, it is to be understood that various changes, even as great as several tenths of one percent in the largest components may be made without departing from the invention.

I claim:

55 1. A heat resistant alloy composed of more than 16% to about 20% aluminum, about 5% to 8.5% chromium, about 0.4% to 1.5% manganese, small amounts of silicon but not more than about 0.25% silicon, and about 0.1% to 0.5% titanium, 60 the balance being substantially all iron.

2. A heat resistant alloy composed of more than 16% to about 20% aluminum, about 5% to 8.5% chromium, about 0.4% to 1.5% manganese, small amounts of silicon but not more than about 65 0.25% silicon, and about 0.1% to 1.5% molybdenum, the balance being substantially all iron.

3. A heat resistant alloy composed of more than 16% to about 20% aluminum, about 5% to 8.5% chromium, about 0.4% to 1.5% manganese, 70 small amounts of silicon but not more than about 0.25% silicon, about 0.1% to 0.5% of at least one of the metals of the group consisting of titanium and molybdenum, the balance being substantially all iron.

75 4. A heat resistant alloy composed of more

than 16% to about 20% aluminum, about 5% to 8.5% chromium, about 0.4% to 1.5% manganese, small amounts of silicon but not more than about 0.25% silicon, about 0.1% to 0.5% titanium, and about 0.5% to 1.5% molybdenum, the balance 5 being substantially all iron.

5. A heat resistant alloy composed of more than 16% to about 20% aluminum, about 5% to 8.5% chromium, about 0.4% to 1.5% manganese, small amounts of silicon but not more than about 10 0.25% silicon, about 0.1% to 0.5% titanium, and not more than 1% molybdenum but sufficient to improve the forgeability and increase the ohmic resistance of the alloy, the balance being substantially all iron. 15

6. A heat resistant alloy composed of more than 16% to about 20% aluminum, about 5% to 8.5% chromium, about 0.4% to 1.0% manganese, small amounts of silicon but not more than about 0.25%, about 0.1% to 0.5% of at least one of the 20 group of elements which consists of titanium and molybdenum, and an additional amount of molybdenum not exceeding a total of about 1.0%, the balance being substantially all iron.

7. A heat resistant alloy composed of more than 16% to about 18% aluminum, about 5% to 8.5% chromium, about 0.4% to 1.0% manganese, about 0.1% to 0.5% titanium, about 0.1% to 1.0% molybdenum, and small amounts of carbon and silicon but not more than about 0.05% carbon and 0.25% silicon, the balance being substantially all iron. 30

8. Heating element consisting of an attenuated body of alloy which is composed of more than 16% to about 20% aluminum, about 5.0% to 35 8.5% chromium, about 0.4% to 1.5% manganese, small amounts of silicon but not more than 0.25%, and about 0.1% to 0.5% of at least one of the metals of the group which consists of titanium and molybdenum, the balance being substantially 40 all iron.

9. Heating element consisting of an attenuated body of alloy which is composed of more than 16% to about 20% aluminum, about 5.0% to 8.5% chromium, about 0.4% to 1.5% manganese, 45 small amounts of silicon but not more than 0.25%, about 0.1% to 0.5% of at least one of the group which consists of titanium and molybdenum, and an additional amount of molybdenum not exceeding a total of about 1.0%, the 50 balance being substantially all iron.

10. Heating element consisting of an attenuated body of alloy which is composed of more than 16% to about 20% aluminum, about 5.0% to 8.5% chromium, about 0.4% to 1.5% manganese, 55 small amounts of silicon but not more than 0.25%, about 0.1% to 0.5% titanium, and about 0.1% to 1.5% molybdenum, the balance being substantially all iron.

11. Heating element consisting of an attenuated body of alloy which is composed of more than 16% to about 20% aluminum, about 5.0% to 8.5% chromium, about 0.4% to 1.5% manganese, small amounts of silicon but not more 65 than 0.25%, about 0.1% to 0.5% titanium, and about 0.1% to 1.0% molybdenum, the balance being substantially all iron.

12. A heat resistant alloy composed of more than 16% to about 20% aluminum, 5% to 8.5% 70 chromium, 0.4% to 1.5% manganese, small amounts of silicon but not more than 0.25%, and a minimum of 0.1% of at least one of the group of elements consisting of titanium and molybdenum, the titanium not exceeding about 0.5% 75

and the molybdenum not exceeding about 1.5%, the balance being substantially all iron.

13. An alloy for electric resistance elements having a specific resistance of at least 200 microhms per centimeter cube, composed of about 16% to 18% aluminum, 5% to 10% chromium, 0.4% to 1.5% manganese, small amounts of carbon and silicon but not more than 0.05% carbon and 0.25% silicon, and about 0.1% to 0.5%

10 titanium, the balance being substantially all iron.

14. An alloy for electric resistance elements having a specific resistance of at least 200 microhms per centimeter cube and a temperature coefficient of resistance approximately equal to zero, composed of about 17.5% aluminum, about 8.5% chromium, about 0.4% manganese, about 0.4% titanium, and silicon but less than 0.25%, the balance being substantially all iron.

HANS JAEGER. 10